

## UNITED STATES PATENT OFFICE

1,944,372

## PROCESS OF PRINTING

George Rivat, Paterson, N. J., assignor to  
Celanese Corporation of America, a corpora-  
tion of Delaware

No Drawing. Application August 2, 1929  
Serial No. 383,173

8 Claims. (Cl. 8—5)

This invention relates to a process of printing yarns and/or fabrics, especially fabrics made of containing organic derivatives of cellulose.

An object of my invention is to apply the principle of discharge printing to fabrics to obtain clear white discharges and colored discharges which do not rub.

Another object of my invention is to utilize vat colors for obtaining discharge prints on fabrics made of or containing cellulose esters or ethers.

A further object of my invention is to effect discharge printing on fabrics made of or containing cellulose derivatives with vat and chrome colors in the presence of a swelling agent and a reducing agent.

Other objects and advantages will appear from the following detailed description.

Heretofore it has been impossible to obtain good clear discharge prints on fabrics utilizing chrome or vat colors. This was particularly true of fabrics made of or containing organic derivatives of cellulose. Clear white discharges on the latter type of fabric were also difficult to obtain.

I have now found that it is possible to secure excellent colored discharges with chrome and/or vat colors if the latter are applied in printing pastes containing suitable reducing agents and agents which will insure thorough penetration of the vat colors. Improved results in white discharges have also been obtained as a result of my invention, which may be described as a super reduction process.

By way of example the invention will be described as applied to fabrics made of or containing cellulose acetate but my process is also applicable to fabrics made of or containing other organic derivatives of cellulose such as cellulose esters (cellulose formate, cellulose propionate) and cellulose ethers (methyl cellulose, ethyl cellulose, etc.). This invention is also applicable to fabrics generally whether the same be made of or contain silk, cotton, wool or artificial silk of the reconstituted cellulose type.

A feature of my invention is the employment of suitable reducing agents in connection with the vat or chrome colors. By a proper selection of the reducing agent and its proper admixture with swelling and penetrating agents, vat colored discharge prints are obtained which are absolutely fixed and which are not rubbed off. Prior to my invention the rubbing of vat color prints was so objectionable that their use for printing purposes was virtually precluded.

This objectionable feature has been overcome by my invention, which may perhaps be best described as a super reduction process. The vat or chrome color is mixed with a suitable thickening

agent such as gum arabic or tragacanth to which is added a swelling agent or agents, such as phenol or alcohol, for the cellulose derivative, reducing agents such as zinc formaldehyde sulfoxylate, sold under the trade-marks Decroline and Protolin, or sodium formaldehyde sulfoxylate, sold under the trade-mark Formopon, and sodium oxalate. Preferably some dithio glycol, sold under the trade-mark Glyazine and caustic soda are also added to the paste, the former acting as a penetrating agent and as a solvent for the vat color. Instead of Glyazine, other glycol derivatives such as thioglycol, ethylene glycol, chlor derivatives of the glycols, triethanolamine, etc. may be used.

To obtain best results, the printing paste with the above ingredients for color discharges, should be allowed to stand at least 24 hours after it is prepared before the same is used. A longer period is preferable since it insures a better reduction of the vat color. I have found that the color has a tendency to rub if the paste is used before the expiration of 24 hours. The prolonged standing of the paste after its preparation apparently results in a better reduction of the color, yielding colored prints which do not rub.

Where chrome colors are employed, the phenol used in the paste should be neutralized, preferably with caustic soda but when vat colors are employed complete neutralization of the phenol is not essential. For white discharges Decroline gives slightly better results than Protolin but the latter is to be preferred where colored discharges are desired.

The following are a few examples of printing pastes which I have found to give excellent results but my invention is not to be considered as limited to these examples.

Examples I and II are for white discharges and examples III and IV are for colored discharges.

## Example I

|                                | Grams per | litre |
|--------------------------------|-----------|-------|
| Decroline                      | 250       | 100   |
| Alcohol                        | 60        |       |
| Phenol                         | 10        |       |
| Water                          | 180       |       |
| Arabic or tragacanth gum (1:1) | 500       | 105   |

## Example II

|                                | Grams per | litre |
|--------------------------------|-----------|-------|
| Protolin                       | 250       |       |
| Phenol                         | 10        |       |
| Alcohol                        | 10        | 110   |
| Pyrogallic acid                | 10        |       |
| Water                          | 180       |       |
| Arabic or tragacanth gum (1:1) | 540       |       |

## Example III

|                                                     | Grams per litre |
|-----------------------------------------------------|-----------------|
| Algol Scarlet G paste (Color Index 1129)<br>reduced | 150             |
| 5 Decroline                                         | 80              |
| Formopon                                            | 20              |
| Water                                               | 60              |
| Phenol                                              | 10              |
| Glyazine                                            | 50              |
| 10 Sodium oxalate                                   | 50              |
| Caustic soda                                        | 40-60           |
| Arabic or tragacanth gum (1:1)                      | 320             |

## Example IV

|                                                     | Grams per litre |
|-----------------------------------------------------|-----------------|
| Algol Scarlet G paste (Color Index 1129)<br>reduced | 150             |
| 20 Protolin                                         | 150             |
| Water                                               | 60              |
| Phenol                                              | 10              |
| Glyazine                                            | 50              |
| Sodium oxalate                                      | 50              |
| Caustic soda                                        | 40-60           |
| 25 Arabic or tragacanth gum (1:1)                   | 320             |

The fabric after being treated with the above pastes in any suitable manner is passed through a Mather Platt for 10 minutes with as much moisture as possible.

30 Although Algol Scarlet G paste (Color Index 1129) is the only vat dye specified in the examples, this invention is not limited to this particular dye. Other vat dyes, especially the anthraquinone vat dyes can be used with excellent results. Also other swelling agents may be employed in place of alcohol.

40 The foregoing detailed description is given merely by way of illustration and many variations may be made therein without departing from the spirit of this invention.

Having described my invention what I claim and desire to secure by Letters Patent is:

1. Method of discharge printing fabric which 45 comprises treating a dyed fabric containing cellulose acetate with a printing paste containing a swelling agent for the fabric under treatment, a vat color and a penetrating agent which is also a solvent for the vat color.

50 2. Method of discharge printing fabric which comprises treating a dyed fabric containing organic derivatives of cellulose with a printing paste containing a reduced vat color, zinc formaldehyde sulfoxylate, a swelling agent for the fabric under treatment, a glycol derivative,

sodium oxalate, caustic soda, and a thickening agent, said paste having been prepared at least twenty four hours before use, and then passing the fabric through a Mather Platt for 10 minutes under moist conditions.

3. Method of discharge printing fabric which comprises treating a dyed fabric containing organic derivatives of cellulose with a printing paste containing a reduced vat color, zinc formaldehyde sulfoxylate, phenol, dithio glycol, sodium oxalate, caustic soda and a thickening agent, and then passing the same through a Mather Platt for 10 minutes under moist conditions.

4. Method of discharge printing fabric which comprises treating a dyed fabric containing cellulose acetate with a printing paste containing a reduced vat color, zinc formaldehyde sulfoxylate, a swelling agent for the fabric under treatment, a glycol derivative, sodium oxalate, caustic soda and a thickening agent, and then passing the same through a Mather Platt for 10 minutes under moist conditions.

5. Method of discharge printing fabric which comprises treating a dyed fabric containing cellulose acetate with a printing paste containing a reduced anthraquinone vat dye, zinc formaldehyde sulfoxylate, a swelling agent for the fabric under treatment, a glycol derivative, sodium oxalate, caustic soda and a thickening agent, and then passing the same through a Mather Platt for 10 minutes under moist conditions.

6. Method of discharge printing fabric which comprises treating a dyed fabric containing cellulose acetate with a printing paste containing a reduced anthraquinone vat dye, zinc formaldehyde sulfoxylate, phenol, dithio glycol, sodium oxalate, caustic soda and a thickening agent, and then passing the same through a Mather Platt for 10 minutes under moist conditions.

7. Method of discharge printing fabric containing an organic derivative of cellulose which comprises treating a dyed fabric with a printing paste containing phenol, a vat color, a penetrating agent which is also a solvent for the vat color and a reducing agent.

8. Method of discharge printing fabric containing an organic derivative of cellulose which comprises treating a dyed fabric with a printing paste containing alcohol, a vat color, a penetrating agent which is also a solvent for the vat color and a reducing agent.

GEORGE RIVAT.